

1

3,290,242

**METAL ANTIOXIDANTS FOR FLUOROESTERS**  
 Harold Ravner, Accokeek, and Carter O. Timmons, Oxon Hill, Md., assignors to the United States of America as represented by the Secretary of the Navy  
 No Drawing. Filed Apr. 18, 1963, Ser. No. 274,064  
 4 Claims. (Cl. 252—26)

The invention described herein may be manufactured and used by or for the Government of the United States of America for governmental purposes without the payment of any royalties thereon or therefor.

This invention relates to fluoroesters, more particularly to improvement in the oxidation stability of fluoroesters at high temperatures.

Developments in military and industrial equipment have presented an increasing demand for lubricants and hydraulic fluids which can meet severe operational requirements. Among such requirements is oxidation stability at high temperatures.

Fluid neutral esters of omega-hydroperfluoroalkylcarbinols and saturated aliphatic hydrocarbon polycarboxylic acids have been heretofore suggested as a source of potential high temperature lubricants and hydraulic fluids. As a class these esters lack the necessary oxidation stability which would allow their use as lubricants or as hydraulic fluids at temperatures in the range of about 400 to 500° F.

It is an object of the present invention to improve the oxidation stability of fluoroesters of the aforesaid class whereby to provide new high temperature lubricants and hydraulic fluids.

We have found certain metals to be antioxidants which impart an exceptional degree of oxidation stability at elevated temperatures in the range of about 400 to 500° F. to fluid neutral esters of omega-hydroperfluoroalkylcarbinols which have from 5 to 11 carbon atoms and saturated aliphatic hydrocarbon di-, tri- and tetracarboxylic acids which have from 3 to 9 carbon atoms in the hydrocarbon groups.

The metals which we have found to be antioxidants for the fluoroesters of the aforesaid group are barium, tin and zinc. The threshold temperature for antioxidant activity of the metals in the fluoroesters is about 400° F. Below this temperature, the fluoroesters are in themselves oxidation stable. The metals are effective as antioxidants even in small concentrations, as low as on the order of from about 0.05 to 0.5% by weight based on the weight of the fluoroesters, to impart a high order of oxidation stability to the fluoroesters at temperatures in the range of from about 400 to 500° F. The antioxidant metal may be brought into contact with the fluoroesters not only in particle form but also in the form of plates or other larger shapes or configurations as found suitable. The surface of the parts of engines or of other mechanisms with which the fluoroesters come into contact, such as oil lines, may consist of the antioxidant metal or a by-pass system may contain the antioxidant metal in the form of a wire mesh or as a confined mass of granules through which the fluoroester flows in contact before returning to areas of lubrications.

The mechanism whereby the metals function as antioxidants in the fluoroesters is not known, but is believed to involve the formation of metal ions in the fluoroesters.

The fluid neutral fluoroesters with which the present invention is concerned may be prepared in known way as described in Ind. Eng. Chem. 48, 445 (1956) from the omega-hydroperfluoroalkylcarbinols of the general formula:



2

wherein  $n$  is an integer from 2 to 5 and aliphatic polycarboxylic acids of the general formula:



5 wherein  $n$  is an integer from 2 to 4 and  $R$  is a saturated aliphatic hydrocarbon group having from 3 to 9 carbon atoms. Thus, the neutral fluoroesters may be derived by the complete esterification of, for example, glutaric, adipic, pimelic, suberic, azelaic, sebacic and undecanedioic acids; methyl succinic, 3-methylglutaric, 1,4-dimethyl adipic, 2,2-dimethyladipic, 1-methyl-4-ethyl adipic acids, etc.; camphoric acid, tricarballylic acid, butane-1,2,4-tricarboxylic acid, butane 1,1,4-tricarboxylic acid, etc., and butane-1,2,4,4-tetracarboxylic acid, butane-1,1,2,3-tetracarboxylic acid, butane-1,1,2,3-tetracarboxylic acid, etc., with fluoroalcohols of the above general formula which are 1H,1H,5H-octafluoro-1-pentanol, 1H,1H,7H-dodecafluoro-1-pheptanol, 1H,1H,9H-hexadecafluoro-1-nonanol and 1H,1H,11H-eicosfluoro-1-undecanol. Illustrative of these fluid neutral fluoroesters are those described in Ind. Eng. Chem. 48, 445, above, for example, bis (1H,1H,5H-octafluoropentyl)- and bis (1H,1H,7H-dodecafluorohexyl) 3-methylglutarates, bis (1H,1H,5H-octafluoropentyl) adipate and sebacate, tri (1H,1H,5H-octafluoropentyl) tricarballylate, etc.

The oxidation stability imparted to the fluoroesters by the metals will vary with the particular metal and fluoroester. It will be higher at the lower temperatures in the aforesaid range since the oxidative stress is less at lower temperatures.

The antioxidant activity of the metals for the fluoroesters may be evaluated in terms of increase in the viscosity and rise in the neutralization number of the fluoroesters and the amount of fluoride evolved from the fluoroesters. The lower the value for these factors, the greater in general the oxidation stability imparted to the fluoroesters by the metals at a given temperature in the aforesaid range. Depending upon the conditions of service use, all or less than all of these factors may govern in the selection of the fluoroesters on the basis of oxidation stability. Thus, where the acid developed in the fluoroester is not a corrosion problem, either by virtue of the acid in itself being non-corrosive or the metal parts with which the fluoroester and developed acid come into contact are acid resistant, rise in the neutralization number can be of minor significance. Similarly, evolved fluoride also can be of minor significance where means are provided for venting of the evolved fluoride from an engine or other system in which the fluoroesters are employed.

Increase in viscosity and rise of the neutralization number of the fluoroesters and the amount of fluoride evolved therefrom on heating the fluoroesters to temperature in the aforesaid range in the presence of the metals may be determined by use of the dynamic oxidation test procedure and apparatus described in Ind. Eng. Chem. 39, 491 (1947). In this test, the samples of the fluoroesters with the metal specimen immersed therein are contained in cylindrical cells made of borosilicate glass. The metal specimens, which may be in the form of strips, are used in clean, degreased condition. The control is a like volume of the fluoroester in a cell but without a metal therein. Each of the cells is equipped with a water-cooled condenser fitted to the top thereof and has a rubber hose connected from the condenser to a separate water trap. Sealed to the upper wall of each of the cells is a means for delivering bubbled air into the bottom of the fluoroester samples in the cells. The cells containing the fluoroester samples and metal specimens and the cell with the control sample are placed in snugly fitting holes in an electrically heated Duralumin block which is thermostatically controlled to hold at the test temperature

$\pm 0.5^\circ$  F. Clean dry air, free from CO<sub>2</sub>, is bubbled through the heated fluoroester samples in the cells at a predetermined volume and rate. The effluent gases from each of the cells which have passed through the individual associated condenser are led into the water trap provided therefor and the fluoride content of the trap liquid determined by the lead chloro-fluoride method. The amount of evolved fluoride is reported as mg. of fluorine per gram of the fluoroester. The viscosity in centistokes at 100° F. and the neutralization number of the fluoroesters are determined before and after the test. The neutralization number is the number of milligrams of potassium hydroxide required to neutralize the fluoroester.

Indicative of the oxidation stability which can be imparted by the metal antioxidants of the invention to the fluoroesters of the aforesaid group at temperatures in the range of 400 to 500° F. are the results obtained on commercial (Du Pont Company) fluid mixed camphorate esters from the complete esterification with camphoric acid of mixed C<sub>5</sub>, C<sub>7</sub> and C<sub>9</sub> fluoroalcohols of the formula H(CF<sub>2</sub>CF<sub>2</sub>)<sub>n</sub>CH<sub>2</sub>OH in which the ratio of the fluoroalcohols was approximately 0.5 mole of the C<sub>5</sub> fluoroalcohol, 1 mole of the C<sub>7</sub> fluoroalcohol and 0.5 mole of the C<sub>9</sub> fluoroalcohol. The mixed camphorate fluoroesters had a microboiling point of 351° C. The tests were conducted at 482° F. for 72 hours using 20 ml. samples of the mixed fluoroesters and metal specimens in the fluoroester samples which generally had surface areas of 10 square centimeters. The air was bubbled into the fluoroester samples in the cells at the rate of 1 cc./gram fluoroester sample/minute. The results of the tests with the several metals as antioxidants are set forth in the following table.

## DYNAMIC OXIDATION TEST

| Metals  | Viscosity Increase at 100° F. (percent) | Neutralization No. Increase | Fluoride Evolved mg. F./gm. |
|---------|-----------------------------------------|-----------------------------|-----------------------------|
| Control | Gelled                                  |                             |                             |
| Barium  | 36                                      | 5.3                         | 2.0                         |
| Tin     | Nil                                     | 3.2                         | 0.45                        |
| Zinc    | 38                                      | 11.0                        | 2.2                         |

Under the conditions of the test, the sample of the mixed fluoroesters which was not protected by a metal antioxidant lost all fluidity, being in the form of a somewhat powdery solid gel at the end of the test period. In contrast, the samples of the mixed fluoroesters which were protected by the metals were still fluid at the end of the test period. The test results show the metals to strongly retard increase in the viscosity of the mixed

fluoroesters at 482° F., tin being outstanding in this respect.

While the invention has been described herein with reference to certain specific embodiments thereof, it obviously may be otherwise practiced without departing from the spirit or scope thereof and, accordingly, such specific embodiments are intended by way of illustration and not in limitation except as may be defined in the appended claims.

What is claimed is:

1. A composition comprising a fluid neutral ester of a fluoroalcohol of the general formula:



15 wherein *n* is an integer from 2 to 5 and an aliphatic polycarboxylic acid of the general formula:



wherein *n* is an integer from 2 to 4 and R is a saturated 20 aliphatic hydrocarbon group having from 3 to 9 carbon atoms and a metal of the group consisting of barium, tin and zinc present therein in amount sufficient to improve the oxidation stability of the fluid neutral ester at temperatures in the range of from about 400° to 500° F.

25 2. A composition as defined in claim 1, wherein the metal is barium.

3. A composition as defined in claim 1, wherein the metal is tin.

4. A composition as defined in claim 1, wherein the 30 fluid neutral ester is a camphorate of at least one fluoroalcohol of the general formula:



wherein *n* is an integer from 2 to 5.

## References Cited by the Examiner

## UNITED STATES PATENTS

2,742,427 4/1956 Reiff ----- 252-56

## FOREIGN PATENTS

610,516 12/1960 Canada.

866,053 4/1961 Great Britain.

## OTHER REFERENCES

45 Mardles: "International Tin Research and Dev. Council," Tech. Publn., Series C #2, pp. 1 to 5 (1934).

Kalichevsky et al.: "Petroleum Refining With Chemicals" (1956), Elsevier Pub. Co., p. 590.

50 Gunderson et al.: "Synthetic Lubricants," Reinhold Pub. Co. (1962), p. 189.

DANIEL E. WYMAN, Primary Examiner.

W. H. CANNON, Assistant Examiner.